

Feb. 7, 1961

A. P. ALEXANDER ET AL

2,970,902

DUCTILE IRON

Filed Jan. 17, 1956

2 Sheets-Sheet 1



250 X Nital & Picral Etch

Fig. 1. Regular Nodular iron 302 brinell.



250X Nital & Picral Etch

Fig. 2. Lanthanum treated nodular iron-197 brinell.



250X Picral & Nital Etch

Fig. 3. Hard nodular iron 363 brinell.

**INVENTORS.**

ADOLPH P. ALEXANDER  
ARTHUR F. SPENGLER, JR.

By *Paulo Riegel*  
ATTY.

Feb. 7, 1961

A. P. ALEXANDER ET AL

2,970,902

DUCTILE IRON

Filed Jan. 17, 1956

2 Sheets-Sheet 2



250 X Picral & Nital Etch

Fig. 4. Same hard nodular iron as  
Fig. 3, with 0.010%  
Lanthanum added - 321 brinell.



250 X Picral & Nital Etch

Fig. 5. Typical structure of  
beneficiated iron produced by  
adding percentages of Lanthanum  
and Magnesium too low for  
complete nodulization.

INVENTORS

ADOLPH P. ALEXANDER  
ARTHUR F. SPENGLER, JR.

By Paul C. Bissel  
ATTY.

# United States Patent Office

2,970,902

Patented Feb. 7, 1961

1

2,970,902

## DUCTILE IRON

Adolph P. Alexander and Arthur F. Spengler, Jr., Memphis, Tenn., assignors to International Harvester Company, a corporation of New Jersey

Filed Jan. 17, 1956, Ser. No. 559,574

9 Claims. (Cl. 75—123)

This invention relates to a new and novel ferrous alloy which may be made from any normal base mix composition of gray iron within commonly known specifications as well as a base mix of gray iron that is not necessarily within the usual range of such specifications. The resulting ferrous alloy, according to this invention, in the "as-cast" condition is soft, ductile, readily machineable and possesses distinct properties of high tensile strength, high elongation and impact strength and thereby produces castings which may be machined without the necessity of a further thermal treatment.

It is well known that castings made from a normal gray iron mix possess free carbon in the form of flaked graphite which is more or less uniformly distributed throughout the matrix resulting in a casting having a low tensile strength in the range of 30,000 to 50,000 pounds per square inch. It is also well known that if magnesium in amounts necessary to introduce from about 0.02 to 0.04 percent in the casting or alternatively cerium in amounts necessary to introduce 0.02 to about 0.050 percent in the casting, or a combination of these two elements, the graphitic carbon tends to coalesce or agglomerate to form particles which are neither flake-like or spherulitic in shape but instead are irregularly shaped in what may be said to be a transition stage between the flake shape on the one hand and spheroidal or spherulitic on the other hand. The particles therefore appear in some portions to resemble an approach to a flake shape and other portions approach that of spheroidal or spherulitic shape. Such an iron is generally termed "beneficiated" in that the resulting castings may possess up to and even exceeding 80,000 pounds per square inch in tensile strength depending upon the percentage of magnesium or cerium, or a combination of both elements, is present in the casting.

However, as is well known, when sufficient amounts of magnesium (i.e. 0.04 to 0.5 percent) or cerium (i.e. 0.05 to 0.5 percent) are added to the molten base gray iron mix resulting in a casting having a percent of magnesium or cerium exceeding the maximum percentages specified above for beneficiated iron, the graphite will essentially coalesce or agglomerate to form nodules of carbon or graphite substantially spheroidal or spherulitic in shape which nodules are more or less disposed uniformly in the matrix in the casting. Such iron is generally termed "nodular" iron and castings made therefrom usually possess a tensile strength in the range of 90,000 to 120,000 pounds per square inch or higher.

It should be mentioned here that the sulphur content of the base gray iron mix used for making beneficiated iron or nodular iron, as above described, must be sufficiently low so that the resulting castings contains a sulphur content of not more than 0.03 percent. If magnesium is used the composition of the base gray iron mix may be hypo-eutectic, eutectic or hyper-eutectic while in the case where cerium is used the base gray iron mix must necessarily be hyper-eutectic. For purposes herein it will be understood that the following well known equation adequately defines the aforementioned terms:

$$CE = TC + \frac{P+Si}{3}$$

2

where TC represents the percent total carbon present in a gray iron casting, P represents the percent phosphorus present and Si represents the percent silicon present. When CE equals 4.30 the iron is said to be of eutectic composition; when CE exceeds 4.30 the iron is said to be of hyper-eutectic composition; and when CE is less than 4.30 the iron is said to be of hypo-eutectic composition.

Gray irons with nodular graphite made as described above from normal base irons that conforms with the requirements of the Society for Automotive Engineers specifications are usually hard and have a Brinell hardness number (3000 kilogram load-10 millimeter ball) above 250 in standard 1 inch thick "Y-Block" test castings illustrated in Military Specification MIL-I-17166A (SHIPS). Castings from these irons in sections of  $\frac{1}{4}$  inch thickness or less are too hard for routine machining operations. In addition these light section castings have sufficient free or massive iron carbides in the matrix of the cast structure to cause the casting to be brittle with little or no ductility. Such castings have a low shock resistance and require thermal treatment for satisfactory engineering use.

Soft as-cast nodular irons can be produced with great difficulty from a cupola with either magnesium or cerium including suitable alloys thereof only if special precautions are taken. One method is to make a base iron having an extremely low silicon content, less than 0.10 percent phosphorus and less than 0.40 percent manganese. Castings made from such base iron would be unsuitable for machining operations. However, if in such a molten base iron mix is added magnesium or cerium in combination with a high amount of silicon and thereafter a further large addition of a silicon alloy is made, a resulting casting may contain from 2.00 to 4.00 percent silicon which would be relatively soft and readily machineable.

For the above reasons it is usual in the foundry industry to use premium priced pig iron or carefully selected expensive steel scrap to use for the production of nodular irons. These requirements for soft as-cast nodular iron make it impractical to economically make gray iron from the same base mix. The only other heretofore known alternative is to make the hard and brittle type nodular iron castings and subsequently subjecting the resulting castings, to a relatively expensive thermal treatment prior to machining operations. It is therefore a prime object of this invention to provide beneficiated and nodular irons which in the as-cast condition are soft and ductile, having high strength and shock resistant properties, and may be made from normal molten base gray iron compositions.

It is a further object of this invention to provide beneficiated and nodular irons which in the as-cast condition are soft and ductile, having high strength and shock resistant properties, and may be made from base gray iron molten mixes having compositions outside the limits of normal gray iron specifications.

A still further object of this invention is to provide beneficiated and nodular irons according to the preceding objects the properties of the castings made therefrom may be further enhanced by a subsequent thermal treatment.

These and other desirable objects inherent in and encompassed by the invention will be more readily understood from the ensuing description, the appended claims and the annexed reproductions of photomicrographs wherein:

Figure 1 is a photomicrograph of a polished and etched surface illustrating hard nodular iron made from a normal base gray iron, the microstructure being enlarged by 250 diameters.

Figure 2 is a photomicrograph of a polished and etched

surface illustrating soft nodular iron made in accordance with this invention using the same base gray iron of Figure 1, the microstructure being enlarged by 250 diameters.

Figure 3 is a photomicrograph of a polished and etched surface illustrating a very hard nodular iron made by the addition of magnesium alloy to a normal base gray iron mix the microstructure being enlarged by 250 diameters.

Figure 4 is a photomicrograph of a polished and etched surface illustrating soft nodular iron made in accordance with this invention using the same base gray iron of Figure 3, the microstructure being enlarged by 250 diameters.

Figure 5 is a photomicrograph of a polished and etched surface illustrating the microstructure of a normal base gray iron beneficiated by the addition of smaller amounts of magnesium and softened in accordance with this invention, the microstructure being enlarged by 250 diameters.

The aforementioned military specification indicates that nodular iron having a silicon content above 2.50 percent is undesirable. It is unusually difficult to produce nodular iron in accordance with the aforesaid military specification which is soft in the as-cast condition from a cupola base iron that is also suitable for pouring gray iron castings conforming to standard engineering specifications because the base iron silicon content must be kept very low to permit a large late addition of ferro-silicon for softening the resulting castings. From this it may be readily appreciated that the production of beneficiated or nodular gray iron castings made from normal base gray iron meeting commonly known engineering specifications would be of exceedingly great value to the foundry industry. Such production would enable a foundry to pour easily machineable castings having tensile strength up to and exceeding 90,000 pounds per square inch. According to our invention this may be accomplished by taking a ladle of molten normal base gray iron, castings of which would have a tensile strength of 30,000 to 50,000 pounds per square inch, and making a simple inexpensive ladle addition of special alloys hereinafter discussed which converts the normal base gray iron to beneficiated or nodular iron of which castings made therefrom will be soft, ductile and of very high tensile strength.

We have discovered that a molten normal base gray iron of hypoeutectic or hyper-eutectic composition, the addition thereto of a mixture of magnesium ferro-silicon (8.5% Mg, 46.0% Si) plus lanthanum, or, magnesium ferro silicon plus a mixture of rare earth metals containing a minimum of 30% lanthanum will result in beneficiated or nodular graphite iron depending upon the amounts added. Thereafter the molten mix is inoculated with a late addition of a graphitizer such as ferro-silicon up to 0.40 percent, and the castings made therefrom are soft and machineable and of high strength properties. By this means we have produced castings having a Brinell hardness number of about 200 on a standard 1" "Y-Block" test bar, with a tensile strength from 80,000 to 100,000 pounds per square inch and, depending upon the silicon content, an elongation of 3 to 10 percent or over.

Nodular graphite iron castings made with lanthanum as outlined above have a hardness range of from only 200 to 225 Brinell in  $\frac{3}{16}$ " thick sections in the as-cast condition. They machined as readily as normal gray irons in the as-cast condition. Chilled areas caused by free carbides were not evident in these light sections. The base gray iron mix for producing these soft as-cast nodular iron castings can be balanced to meet any American Society for Testing Materials specifications for gray iron from 110 to 122 as described in ASTM Designation A159-49T which covers gray irons having tensile strength in the range from 20,000 to 45,000 pounds per square inch.

The above described results are exceedingly unusual for nodular graphite irons because castings made from the same base irons mentioned above but in accordance with previously known methods or compositions would result in castings having a Brinell hardness of over 250 in test bars and light or thin section castings could be machined only with great difficulty if at all.

Referring now to Figures 1 and 2 these photomicrographs illustrate the structures of nodular irons made from the same gray iron base mix with the addition of magnesium which formed the spherulitic or nodular graphite particles. However in the case of Figure 2 the molten iron was in further addition treated with lanthanum in accordance with our invention. The Brinell hardness of the casting illustrated in Figure 1 was 302 while that shown in Figure 2 was only 197. A comparison of the two microstructures indicates that considerable more graphite carbon was freed to form nodules when lanthanum was present resulting in a casting having far more ferrite in the matrix. Thus it seems that the lanthanum reduces the dissolved carbon or combined carbon to form additional graphite nodules thereby resulting in a softer casting.

As a specific example of the above described results we present a comparison of nodular iron, made by a well known procedure, with nodular iron made in accordance with this invention. Four hundred pounds of basic cupola normal gray base iron was used. To the first lot of two hundred pounds was added 2.25 percent magnesium ferro-silicon (8.5% Mg, 46.0% Si) containing 0.50 percent cerium plus 75 grams of a "high cerium rare earth alloy" (Misch-metal, see Table 1). Then the first lot was inoculated with 0.35% ferro-silicon (75% Si) and poured into castings. The second lot was made identically the same as the first lot except instead of the "high cerium rare earth alloy" 75 grams of "high lanthanum rare earth alloy" (see Table 1) was substituted. Analysis of the castings of the first lot indicated about 0.003 percent lanthanum present while that of the second lot showed about 0.010 percent lanthanum present.

TABLE 1  
*Analysis of rare earths*

|       | High Cerium (Misch-Metal), percent | High Lanthanum |
|-------|------------------------------------|----------------|
| Ce    | 45                                 | 45-50%         |
| La    | 25                                 | 30% (Mln.)     |
| Nd-Pr | 15                                 |                |
| Sm    | 10                                 |                |
| Dld   |                                    | 20-24%         |
| Fe    | 5                                  | 1.0% (Max.)    |

<sup>1</sup> Dld. Group of rare earths having atomic numbers 59 to 71 inclusive and 39 in varying amounts.

The castings made from the above mentioned two lots were tested for hardness and the results are shown in Table 2.

TABLE 2

*Standard 1" "Y-Block" hardness<sup>1</sup> of high cerium and high lanthanum nodular in as-cast condition*

|     | First Lot              | Second Lot                |
|-----|------------------------|---------------------------|
|     | High Cerium Rare Earth | High Lanthanum Rare Earth |
| 277 | 197                    |                           |
| 269 | 197                    |                           |
| 262 | 197                    |                           |

<sup>1</sup> Brinell hardness no. (3,000 kg. Load-10 mm. ball).

The Brinell hardness test results of the first lot shown in Table 2 are typical and are in conformance with the results reported by others. However, the Brinell hardness test results of the second lot are unusually low and illustrates the effect of our invention in softening or ductilizing the resulting nodular iron. The same type of striking results are obtained in the case of beneficiated irons too. In the case of the castings from the second lot the microstructures thereof again showed that far more ferrite (approximately 80%) was present than that of the castings from the first lot. Furthermore the Brinell hardness of the nodular graphite iron made with the magnesium without the addition of rare earth material was over 250. Thus it can be seen that increasing amounts of magnesium or cerium in the castings results in progressive hardening or, in other words, the presence of cerium or magnesium in iron castings will result in a harder and more brittle product.

The above discussed first example was concerned primarily with a comparison of hardness characteristics of nodular iron made in accordance with previous known concepts with that of the addition of lanthanum according to our invention.

Table 3 illustrates, in a series of nodular irons made from normal base gray irons, the effect of composition on certain physical properties of the resulting castings made therefrom. It may be noted that the elongation property decreases as the silicon content increases while the tensile strength remains fairly constant at from 92,000 to 95,000 pounds per square inch after 2.75% silicon is reached.

TABLE 3

*As-cast properties of nodular iron produced by additions of high lanthanum rare earths and magnesium*

| Heat No.                          | 1      | 2      | 3      | 4      | 5      | 6      |
|-----------------------------------|--------|--------|--------|--------|--------|--------|
| Si, percent                       | 2.47   | 2.51   | 2.74   | 2.81   | 3.21   | 3.56   |
| T.C., percent                     | 3.44   | 3.51   | 3.53   | 3.21   | 3.21   | 2.82   |
| Mn, percent                       | 0.41   | 0.39   | 0.45   | 0.44   | 0.47   | 0.45   |
| P, percent                        | 0.05   | 0.04   | 0.04   | 0.05   | 0.06   | 0.08   |
| S, percent                        | 0.02   | 0.02   | 0.02   | 0.02   | 0.02   | 0.02   |
| Ni, percent                       | 0.12   | 0.15   | 0.31   | 0.23   | 0.27   | 0.18   |
| Cr, percent                       | 0.07   | 0.10   | 0.13   | 0.16   | 0.11   | 0.17   |
| Mg, percent                       | 0.045  | 0.055  | 0.043  | 0.047  | 0.053  | 0.065  |
| Ce, percent                       | 0.023  | 0.026  | 0.015  | 0.019  | 0.022  | 0.019  |
| La, percent                       | 0.009  | 0.011  | 0.007  | 0.008  | 0.009  | 0.009  |
| BHN                               | 197    | 197    | 200    | 207    | 197    | 229    |
| Tensile (p.s.i.)                  | 79,500 | 84,500 | 92,000 | 95,000 | 91,900 | 92,000 |
| Yield (p.s.i.)                    | 61,200 | 63,600 | 81,250 | 76,500 | 66,450 | 79,600 |
| Elongation, percent               | 10     | 11     | 8.5    | 17.0   | 7.0    | 3.0    |
| Unnotched Charpy Impact, Ft. lbs: |        |        |        |        |        |        |
| 70° F                             |        |        | 21.8   | 19.0   | 11.0   | 4.5    |
| -40° F                            |        |        | 8.3    | 5.5    | 5.5    | 3.0    |

<sup>1</sup> Broke outside gauge marks.

A rise in tensile strength to about 80,000 to 95,000 pounds per square inch at constant hardness is rather unusual in nodular iron and even in steel. This unusual result seems to be associated with the effect of the presence of lanthanum according to this invention which will be discussed later. It should also be noted from Table 3 that the silicon and carbon contents of the several heats vary considerably but the softening effect of the lanthanum appears to control the hardness at a low constant. In respect of hardness we have also noted a rather amazing phenomena in lanthanum softened nodular iron. We find that light section castings as thick as  $\frac{3}{16}$ " are softer as cast than the standard 1" thick "Y-Block" corresponding test bar. As an example we found that using the same iron a "Y-Block" 1" thick exhibited a hardness of 241 Brinell while a  $\frac{3}{16}$ " thick casting of the same iron composition showed only 217 Brinell.

Impact strength of lanthanum treated nodular irons are also of a higher order than that of previously known

nodular irons. As shown in Table 5 the enhanced impact strength of nodular irons made in accordance with our invention appears to be independent of the base composition of the iron or, in other words, the softening effect of the lanthanum and its effect on raising impact strength of nodular iron is, at least to an appreciable extent, independent of the composition of the base iron which may be of either hypo-eutectic or hyper-eutectic composition.

10 In nodular or beneficiated graphite iron the elongation properties vary inversely with the phosphorus content. Therefore the phosphorus content should be kept below 0.1 percent to obtain good elongation properties. It is also preferable to keep the percentage content of certain other elements such as silicon, manganese, nickel, etc., low in the iron for maximum ductility of the resulting casting. However, if special characteristics such as high strength or wear resistance are required, the nodular or beneficiated iron may be deliberately alloyed in a well known manner. In these cases the incorporation of lanthanum of this invention will soften the iron and will increase the impact resistance.

25 The effect of thermal treatment on lanthanum containing nodular iron castings made according to this invention is illustrated in Table 4 for heat Nos. 3 to 6 of Table No. 3.

TABLE 4

*Heat treated properties of nodular iron produced by additions of high lanthanum rare earths and magnesium as in Table 2*

| Heat No.          | 3                                                                                                | 4       | 5       | 6       |         |
|-------------------|--------------------------------------------------------------------------------------------------|---------|---------|---------|---------|
| <b>Treatment:</b> |                                                                                                  |         |         |         |         |
| 40                | Short Cycle Anneal, 1,700° F., 2 $\frac{1}{2}$ Hr., Air Cool—                                    |         |         |         |         |
|                   | Tensile                                                                                          | 70,500  | 73,000  | 69,700  | 80,200  |
|                   | Yield                                                                                            | 58,100  | 56,400  | 56,800  | 63,500  |
|                   | Elong., 2"                                                                                       | 19.0    | 21.0    | 23.0    | 17.0    |
|                   | Hardness, BHN                                                                                    | 179     | 179     | 170     | 197     |
|                   | Charpy Impact:                                                                                   |         |         |         |         |
|                   | 70° F                                                                                            | 57.5    | 68.0    | 67.5    | 29.0    |
|                   | -40° F                                                                                           | 5.5     | 13.0    | 29.0    | 7.0     |
| 45                | 1,400° F., 3 Hrs., Air Cool—                                                                     |         |         |         |         |
|                   | Tensile                                                                                          | 77,500  | 84,000  | 76,850  | 81,000  |
|                   | Yield                                                                                            | 57,100  | 64,100  | 58,300  | 68,250  |
|                   | Elong., 2"                                                                                       | 15.0    | 12.5    | 18.5    | 17.2    |
|                   | Hardness, BHN                                                                                    | 187     | 217     | 187     | 207     |
|                   | Charpy Impact:                                                                                   |         |         |         |         |
|                   | 70° F                                                                                            | 60.8    | 12.5    | 36.5    | 34.0    |
|                   | -40° F                                                                                           | 15.8    | 6.0     | 11.0    | 5.5     |
| 50                | Oil Quench and Temper, 1,725° F., 2 $\frac{1}{2}$ Hrs.; Temper, 1,100° F., 2 $\frac{1}{2}$ Hrs.— |         |         |         |         |
|                   | Tensile                                                                                          | 151,000 | 149,000 | 152,500 | 122,000 |
|                   | Yield                                                                                            | 127,500 | 119,000 | 122,000 | 110,500 |
|                   | Elong., 2"                                                                                       | 2.5     | 3.0     | 3.5     | 4.0     |
|                   | Hardness, BHN                                                                                    | 363     | 363     | 363     | 241     |
|                   | Charpy Impact:                                                                                   |         |         |         |         |
|                   | 70° F                                                                                            | 21.0    | 17.5    | 28.0    | 17.5    |
|                   | -40° F                                                                                           | 14.0    | 11.5    | 16.0    | 10.5    |
| 60                | Normalize, 1,700° F., 2 $\frac{1}{2}$ Hrs., Air Cool—                                            |         |         |         |         |
|                   | Tensile                                                                                          | 114,500 | 111,800 | 114,000 | 109,250 |
|                   | Yield                                                                                            | 90,000  | 91,750  | 92,500  | 85,250  |
|                   | Elong., 2"                                                                                       | 4.5     | 3.0     | 3.5     | 5.0     |
|                   | Hardness, BHN                                                                                    | 269     | 302     | 285     | 269     |
|                   | Charpy Impact:                                                                                   |         |         |         |         |
|                   | 70° F                                                                                            | 16.5    | 10.0    | 14.5    | 16.5    |
|                   | -40° F                                                                                           | 9.5     | 9.0     | 8.5     | 8.5     |

65 The above results from thermal treatment appear to be well in line with that which might be reasonably expected.

70 Although Charpy impact test results apparently do not establish iron toughness as a criterion which is more thoroughly discussed in Designation E23-47T of the American Society for Testing Materials, nevertheless we tested some of the nodular iron castings of this invention for comparison with nodular irons of the well known type. These impact test results are shown in Table 5.

7  
TABLE 5Impact results on standard<sup>1</sup> nodular iron and nodular iron treated with lanthanum<sup>2</sup>

| Type            | Silicon, Percent | As Cast Impact, Ft. Lbs. <sup>3</sup> |         | 5 Hr. Anneal <sup>2</sup> Impact, Ft. Lbs. |         |
|-----------------|------------------|---------------------------------------|---------|--------------------------------------------|---------|
|                 |                  | 70° F.                                | -40° F. | 70° F.                                     | -40° F. |
| Standard.....   | 2.81             | 9.2                                   | 4.3     | 52.5                                       | 13.0    |
| Do.....         | 2.75             | 15.0                                  | 8.5     | 85.0                                       | 75.0    |
| Do.....         | 3.04             | 11.0                                  | 5.0     | 25.5                                       | 18.5    |
| La Treated..... | 2.74             | 21.8                                  | 8.3     | 57.5                                       | 5.5     |
| Do.....         | 2.81             | 19.0                                  | 5.5     | 68.0                                       | 13.0    |
| Do.....         | 3.21             | 11.0                                  | 5.5     | 67.5                                       | 29.0    |

<sup>1</sup> Gray Iron base treated with magnesium and silicon alloy.<sup>2</sup> Similar base iron treated with magnesium and silicon alloy plus high lanthanum rare earth alloy.<sup>3</sup> Charpy unnotched impact as per A.S.T.M. E23-47T.<sup>4</sup> 2½" hrs., 1700° F.-2½ hrs. 1400° F., air cooled total time, 5 hrs. (standard production cycle).

As might be expected the impact test results in Table 5 are quite scattered. The single extremely high result for standard nodular iron is not accounted for nor was it duplicated. Disregarding this extremely high result it appears that the lanthanum treated nodular iron made in accordance with this invention may have an average impact strength of somewhat higher order than that possessed by nodular iron made in accordance with previously known methods.

As a further demonstration of the softening effect in the as-cast condition of nodular graphite iron by "high lanthanum rare earths" containing a minimum of 30 percent lanthanum, standard nodular iron was first made by the well known addition of magnesium alloys. The hardness of a standard 1" thick Y-Block test bar casting was 302 Brinell. To a 200 pound quantity of the same melt an amount of "high lanthanum rare earths" was added to incorporate one-fourth ounce of lanthanum and the resulting hardness of a 1" thick Y-Block casting was only 250 Brinell. Then in another similar type test a very hard type of nodular iron was made which resulted in castings having a Brinell hardness of 363 (Figure 3). Then to 200 pounds of the iron melt was added only 8 grams of elemental lanthanum. The resulting castings had but 0.010 percent lanthanum and the Brinell hardness dropped to 321 (Figure 4).

Comparing the microstructures of the two irons made in the last described test as shown in Figures 3 and 4, it will again be noted that the lanthanum containing iron (Figure 4) shows more carbon in the form of graphite nodules than that shown in the untreated iron of Figure 3. Again it appears that the lanthanum tends to free more carbon to form nodules and correspondingly increasing the amount or percentage of ferrite present in the matrix.

The underlying causes and reasons for the formation of nodular graphite instead of flake graphite in iron is not yet thoroughly understood. Also the reason for the softening effect by lanthanum is not completely clear. As stated previously there is some evidence that lanthanum frees an additional amount of carbon to form more graphite nodules and thereby increase the amount of ferrite present in the matrix through reduction of carbides. It is also suspected that lanthanum softens the iron by combining with gases such as hydrogen, oxygen and nitrogen which are well known potent iron hardeners.

It has been mentioned previously that the presence of cerium or magnesium will result in a harder gray iron in the as-cast condition. It should also be noted that under certain circumstances lanthanum may be a hardener for gray iron. It has been found during the course of our investigation that if the amount of lanthanum in the iron exceeds 0.020 percent the resulting iron will progressively become harder as the percentage of lanthanum further increases. Therefore only minute percentages of lan-

thanum should be used to soften gray iron, namely, the range of 0.004 to 0.020 percent lanthanum, to soften either beneficiated or nodular iron.

As the percentage of magnesium is lowered to below about 0.03 or 0.04 percent and the lanthanum below 0.004 percent complete spheroidization of the graphite is not achieved and the resulting product is of the beneficiated iron type previously discussed. Figure 5 represents a typical structure of beneficiated iron which in this illustration has but relatively few nodules, the bulk of the free carbon being coalesced to a transitional stage between flake form and nodular form. Such beneficiated iron is soft having a tensile strength in the order of 80,000 pounds per square inch and may have an elongation of up to and even exceeding six percent. For example a beneficiated iron made in accordance with the above and shown in Figure 5 possessed, in the as-cast condition, a tensile strength of 81,000 pounds per square inch with a yield strength of 61,000 pounds per square inch and an elongation of 4 percent. Such iron may be used in numerous applications without the necessity of supplemental thermal treatments.

Having thus described our invention including several specific examples thereof it can now be seen that the objects of the invention have been fully achieved and it must be understood that changes and modifications might be made which do not depart from the spirit of the invention as disclosed nor from the scope thereof as defined in the appended claims.

30 We claim:

1. A ductile iron casting having improved machinability characteristics containing in the matrix thereof particles of carbon substantially in agglomerated form, said casting containing from 3.00 to 3.70% total carbon, from 1.80 to 2.80% silicon, from 0.50 to 1.00% manganese, from 0.10 to 0.25% phosphorus, not more than 0.03% sulfur, a carbon agglomerant retained in an amount sufficient to agglomerate substantially said carbon particles in the absence of effective amounts of retained residual elements subversive to said carbon agglomerant, and a ductilizing agent consisting of metallic lanthanum retained in an amount of 0.004 to 0.020 percent to impart said improved machinability characteristics to said casting in the as-cast condition.

2. A ductile iron casting having improved machinability characteristics containing in the matrix thereof particles of carbon agglomerated substantially in spheroidal form, said casting containing from 3.00 to 3.70% total carbon, from 1.80 to 2.80% silicon, from 0.50 to 1.00% manganese, from 0.10 to 0.25% phosphorus, not more than 0.03% sulfur, a carbon agglomerant retained in an amount from 0.02 to 0.50% selected from the group of metals consisting of cerium and magnesium in the absence of effective amounts of retained residual elements subversive to said carbon agglomerant, and a ductilizing agent consisting of metallic lanthanum retained in an amount of 0.004 to 0.020 percent to impart said improved machinability characteristics to said casting in the as-cast condition.

3. A ductile iron casting having improved machinability characteristics containing in the matrix thereof particles of carbon agglomerated substantially in spheroidal form, said casting containing from 3.00 to 3.70% total carbon, from 1.80 to 2.80% silicon, from 0.50 to 1.00% manganese, from 0.10 to 0.25% phosphorus, not more than 0.03% sulfur, a retained carbon agglomerant selected from the group of metals consisting of magnesium in an amount from 0.04 to 0.5% and cerium in an amount from 0.05 to 0.50% in the absence of effective amounts of retained residual elements subversive to said carbon agglomerant, and a ductilizing agent consisting of metallic lanthanum retained in an amount from 0.004 to 0.020 percent to impart said improved machinability characteristics to said casting in the as-cast condition.

4. A ductile iron casting having improved machinability

ty characteristics containing in the matrix thereof particles of agglomerated graphite shaped irregularly in a transition stage between flake form and spherulitic form, said casting containing from 3.00 to 3.70% total carbon, from 1.80 to 2.80% silicon, from 0.50 to 1.00% manganese, from 0.10 to 0.25% phosphorus, not more than 0.03% sulfur, a retained graphite agglomerant selected from the group of metals consisting of magnesium in an amount from 0.02 to 0.04% and cerium in an amount from 0.02 to 0.05% in the absence of effective amounts of retained residual elements subversive to said graphite agglomerant, and a ductilizing agent consisting of metallic lanthanum retained in an amount from 0.004 to 0.020 percent to impart said improved machinability characteristics to said casting in the as-cast condition.

5. A ductile iron casting having improved machinability characteristics containing in the matrix thereof particles of carbon substantially in agglomerated form, said casting containing from 2.82 to 3.53% total carbon, from 2.47 to 3.56% silicon, not more than 0.1% phosphorus, not more than 0.03% sulfur, a carbon agglomerant retained in an amount sufficient to agglomerate substantially said carbon particles in the absence of effective amounts of retained residual elements subversive to said carbon agglomerant, and a ductilizing agent consisting of metallic lanthanum retained in an amount of 0.004 to 0.020 percent to impart said improved machinability characteristics to said casting in the as-cast condition.

6. A ductile iron casting having improved machinability characteristics containing in the matrix thereof particles of carbon agglomerated substantially in spheroidal form, said casting containing from 2.82 to 3.53% total carbon, from 2.47 to 3.56% silicon, not more than 0.1% phosphorus, not more than 0.03% sulfur, a carbon agglomerant retained in an amount from 0.02 to 0.50% selected from the group of metals consisting of cerium and magnesium in the absence of effective amounts of retained residual elements subversive to said carbon agglomerant, and a ductilizing agent consisting of metallic lanthanum retained in an amount of 0.004 to 0.020% to 40 impart said improved machinability characteristics to said casting in the as-cast condition.

7. A ductile iron casting having improved machinability characteristics containing in the matrix thereof particles of carbon agglomerated substantially in spheroidal form, said casting containing from 2.82 to 3.53% total carbon, from 2.47 to 3.56% silicon, not more than 0.1% phosphorus, not more than 0.03% sulfur, a retained carbon agglomerant selected from the group of

metals consisting of magnesium in an amount from 0.04 to 0.50% and cerium in an amount from 0.05 to 0.50% in the absence of effective amounts of retained residual elements subversive to said carbon agglomerant, and a ductilizing agent consisting of metallic lanthanum retained in an amount from 0.004 to 0.020 percent to impart said improved machinability characteristics to said casting in the as-cast condition.

8. A ductile iron casting having improved machinability characteristics containing in the matrix thereof particles of agglomerated graphite shaped irregularly in a transition stage between flake form and spherulitic form, said casting containing from 2.82 to 3.53% total carbon, from 2.47 to 3.56% silicon, not more than 0.1% phosphorus, not more than 0.03% sulfur, a retained graphite agglomerant selected from the group of metals consisting of magnesium in an amount from 0.02 to 0.04 and cerium in an amount from 0.02 to 0.05% in the absence of effective amounts of retained residual elements subversive to said graphite agglomerant, and a ductilizing agent consisting of metallic lanthanum retained in an amount from 0.004 to 0.020 percent to impart said improved machinability characteristics to said casting in the as-cast condition.

9. A ductile iron casting having improved machinability characteristics containing in the matrix thereof particles of carbon agglomerated substantially in spheroidal form, said casting containing from 2.82 to 3.53% total carbon, from 2.47 to 3.56% silicon, not more than 0.1% phosphorus, not more than 0.03% sulfur, a retained carbon agglomerant selected from the group of metals consisting of magnesium in an amount from 0.04 to 0.50% and cerium in an amount from 0.05 to 0.50% in the absence of effective amounts of retained residual elements subversive to said carbon agglomerant, and a ductilizing agent consisting of metallic lanthanum retained in an amount from 0.007 to 0.011% to impart said improved machinability characteristics to said casting in the as-cast condition.

#### References Cited in the file of this patent

##### UNITED STATES PATENTS

|           |                |               |
|-----------|----------------|---------------|
| 2,622,022 | Crome          | Dec. 16, 1952 |
| 2,841,490 | Stevens et al. | July 1, 1958  |

##### FOREIGN PATENTS

|           |               |               |
|-----------|---------------|---------------|
| 721,717   | Great Britain | Jan. 12, 1955 |
| 730,712   | Great Britain | May 25, 1955  |
| 1,070,939 | France        | Aug. 19, 1954 |